

# UNITED STATES PATENT OFFICE.

MORITZ FREIBERGER, OF BUDAPEST, AUSTRIA-HUNGARY.

## PROCESS OF PRODUCING PATTERNS ON FABRICS.

**1,080,433.**

Specification of Letters Patent.

Patented Dec. 2, 1913.

No Drawing.

Application filed August 10, 1908. Serial No. 447,879.

*To all whom it may concern:*

Be it known that I, MORITZ FREIBERGER, residing at 11 Lajos utca 174, Budapest, in the Empire of Austria-Hungary, have invented certain new and useful Improvements in Processes of Producing Patterns on Fabrics, of which the following is a specification.

The present invention relates to a process of producing patterns on fabrics.

The nitrogen oxy-acids are capable, owing to their oxidizing properties, of destroying certain dyestuffs, or altering their color. Thus for instance indigo, even of dark tints, may be discharged by printing on it nitric acid. This method, however, is very rarely employed, because nitric acid renders it impossible to use metallic printing-blocks or metallic printing-rollers and affects the firmness of the fiber, a fact which prohibits an extensive use of the said product in the industry.

Now I have found a process by which it is possible to utilize the oxidizing action of the said compounds for discharging dyestuffs in a satisfactory manner without causing a corrosion of the fiber. This process consists in applying to the fabric the color of which is to be discharged, printing colors which contain salts of the nitrogen oxy-acids that cannot injure the metallic printing rollers, and in effecting the discharging action by subsequently passing the fabrics through an acid bath. In this process it is important that the acid bath should be prepared at such a concentration and temperature that the duration of the passage of the fabric may be as short as possible whereby a complete discharging is obtained without affecting the fiber.

There may be used as discharging agents the salts of nitric acid, nitrous acid and hyponitrous acid, as well as the salts of the analogous acids derived from the said three acids. Strong acids, particularly sulfuric acid, and acid salts may be employed as the components of the acid bath, these liberating the acid from the salts of the above mentioned compounds, the liberated acid becoming the discharging agent. Thus, to illustrate my process, the fabric may be previously dyed with any desired color, then, in accordance with the pattern to be produced, it is printed with a salt of the nitrogen oxy-acid desired to effect the discharg-

ing action. The fabric is then exposed to as short a passage through an acid as is sufficient for causing the reaction between the salt and the acid but does not permit of any harmful action of the acid on the fabric. The previously applied dye will then be discharged or has its color altered at the places printed with the salt, as at these places free nitrogen oxy-acid is produced. Thus for example, if it is desired to produce on a blue ground a pattern formed of white, yellow and red elements, a fabric dyed in indigo and eventually prepared in naphthol is printed with nitrate of zinc or with nitrite of soda to obtain white, with nitrate of lead to obtain yellow, and with nitrate of soda to obtain red, with which latter salt, however, developing colors or red body colors or dyestuffs are mixed. The fabric is then steamed, exposed for a few seconds to a passage through sulfuric acid at 40° Baumé, washed and then treated in chromate of potassium for developing the yellow color.

By combining the discharging color with dyestuffs, or with compounds from which colors can be produced, colored effects, so-called "colored discharges" may be obtained. Further by adding a reducing agent, which frequently increases the discharging action in a surprising manner, a consecutive reducing and oxidizing action may be produced on one and the same spot of the fiber. In this case the passage through the acid bath must be preceded by steaming which causes the reducing-agent to act. By this procedure quite new and peculiar effects can be obtained.

The process may be illustrated by the following examples:

Example I: The following discharge, namely: 200 grams of nitrate of zinc, 1 kg. of starch paste, is printed on an indigo-ground, and after drying, the fabric is passed for a few seconds through sulfuric acid of 40 Bé. at 50-80° C. It is then washed, passed through caustic soda lye of 1° Bé. for half a minute at 40° C. and again washed and dried.

Example II: Like Example I with the exception that: 200 grams of sodium nitrite, and 200 grams of starch paste are used for discharging.

Example III: The discharge described in Example II is passed for a few seconds at 80° C. through a bath consisting of: 300

110

liters of water, 100 kg. of sulfuric acid of 66 Bé., 100 kg. of hydrochloric acid of 20° Bé., 30 kg. of oxalic acid.

Example IV: The fabric previously prepared in the known manner with naphthol (20 grams of naphthol R., 40 ccm. of caustic soda lye of 22° Bé., and 20 grams of Para soap (sodium or ammonia-soap of ricinoleic acid) per liter of the preparing bath) is printed with the discharging colors, passed through sulfuric acid of 40° Bé. for a few seconds at 50-80° C. and dried.

*Discharge-white.*—200 grams of nitrate of zinc, 1 kg. of starch paste, 20 grams of concentrated formic acid.

*Discharge-yellow.*—200 grams of nitrate of lead, 1000 grams of tragacanth water.

*Discharge-red.*—Paranitranilin red-printing-color containing 16 grams of paranitranilin and 200 grams of sodium nitrate added per liter of the printing color. For developing the yellow (chrome-yellow) the fabric is treated with chromate of potassium in the usual manner and then slightly soaped as may be required.

Example V: The fabric naphtholated according to Example IV is printed with the following: "Yellow-discharge" 150 grams of nitrate of lead, 60 grams of hydrosulfite N. F. concentrated, 1 kg. of starch paste. The fabric is then printed over with the discharge-red, made according to Example IV, and passed through the "Mather Platt". The further treatment is carried out according to Example IV. Thus yellow in combination with red and blue is obtained, the red discharging thereby the blue.

Example VI: Indigo-dyed cloth is topped with cresotin-yellow G. or aurophenin O. This green dyeing is printed with the discharge-white described hereafter, treated in the Mather Platt, passed through sulfuric acid according to Example I and finished.

45 *Discharge-white color.*—100 grams of nitrate, 100 grams of hydrosulfite N. F. concentrated, 8 grams of anthraquinone paste, 1 kg. of starch paste.

Example VII: According to Example VI, the indigo dyed cloth however being topped in the usual manner with paranitranilin red instead of with direct dyestuffs.

I claim—

1. The process of figuring fabrics, which 55 consists in applying to the fabric, in either sequence, a dyestuff giving the ground color, and a salt of an oxy-acid of nitrogen, said salt being printed on, and reacting on said

salt with an acid reagent under conditions to discharge the color.

2. The process of figuring fabrics, which consists in applying to the fabric, in either sequence, a dyestuff giving the ground color, and a salt of an oxy-acid of nitrogen, said salt being printed on, and reacting on said salt with hot, strong, sulfuric acid under conditions to discharge the color.

3. The process of producing patterns on fabrics, dyed with a ground color, which consists in printing on the fabric with a salt of a nitrogen oxy-acid, then subjecting the fabric thus treated to the action of a strong acid, and then washing the fabric.

4. The process of producing patterns on fabrics, dyed with a ground color, which 75 consists in printing discharges comprising salts of the nitrogen oxy-acids, then subjecting the fabric thus treated to the action of a strong acid to set free the nitrogen oxy-acid in the fiber, and then washing the fabric.

5. The process of producing patterns by means of nitrogen oxy-acids on fabrics dyed with a ground color without affecting the firmness of the fiber, which consists in causing the salts of the nitrogen oxy-acids 85 printed on the fabric to act by means of a short treatment with hot and strong acids.

6. The process of producing patterns by means of nitrogen oxy-acids on fabrics dyed with a ground color without affecting the 90 firmness of the fiber, which consists in causing the salts of the nitrogen oxy-acids printed on the fabric and to which, for the purpose of producing multi-colored effects, dyestuffs are added, to act by means of a 95 short treatment with hot and strong acids.

7. The process of producing patterns on fabrics, dyed with a ground color, which consists in printing on the fabric a mixture 100 consisting of a salt of a nitrogen oxy-acid and a substance capable of forming colors on the fiber, then subjecting the fabric thus treated to the action of a strong acid, and washing the fabric.

8. The process of producing patterns on 105 fabrics dyed with a ground color, which consists in printing on the fabric a salt of nitric acid, then subjecting the fabric thus treated to the action of a strong acid, and washing the fabric.

In testimony whereof I affix my signature in presence of two witnesses.

MORITZ FREIBERGER.

Witnesses:

E. F. KELEMEN,  
MICHAEL WINORTH.